

UNITED STATES PATENT OFFICE

2.225.352

# **MOTHPROOFING COMPOUND AND METHOD OF USING**

Lawrence W. Roberts, Philadelphia, Pa.

No Drawing. Application November 25, 1936,  
Serial No. 112,706

**6 Claims. (Cl. 167—37)**

This invention relates to mothproofing of fabrics and to mothproofing and moth-repelling compounds to be used in connection therewith. It has heretofore been proposed to treat fabrics with silicofluorides, in order to mothproof them, but for one reason or another the known compositions have not proved entirely satisfactory. For another thing, when sprayed onto the material they have not penetrated sufficiently to render the material mothproof for more than about a year. Also, it has proved difficult to provide a composition in which the fabric can be immersed without resulting in an uneven color or streaking in the finished material, or an objectionable "hand." Many other difficulties arise in the practical application of mothproofing compositions to fabrics, as is well understood by those skilled in the art.

With all these various considerations in mind, it may now be explained that the substances and solutions or suspensions to be applied, for the purpose of my invention, comprise, broadly speaking, a silicofluoride having a relatively high water-solubility, a double salt of antimony, a coating mordant and such other adjuvant materials as the particular conditions may require.

Magnesium and ammonium silicofluorides have been found very efficient in this connection because of their high solubility and relatively high adsorbability to the fabrics in conjunction with appropriate mordanting agents. Other silicofluorides of good water-solubility are also available. When used alone, these salts are apt to be lost either by dusting off from the treated fabrics or during subsequent steaming or cleaning of made-up fabrics or garments, etc., hence the necessity of appropriately balanced fixing agents.

agents.

40 Silicofluorides, in general, have been recommended as protective agents against moths, but in practice, especially under conditions of the art in industrial practice as herein discussed, impregnation with such silicofluorides alone does not have the full practical value which a truly protective agent should possess under all the varying conditions of mill practice.

45

In order to retain the mothproofing effect of such silicofluorides, it is important that they be fixed upon the fibres by a suitable agent having mordant properties. Such mordanting effects are attained, for the multiple purposes of this invention, by an appropriate relative quantitative adaptation of suitable water-soluble materials which will have selective properties both as affecting the "hand" or "feel" of the material, moth repulsion, and fixing. Thus, by way of illustration, aluminum sulphate, or an equivalent salt, in the present invention, performs the double function of a fixing agent for the chosen silicofluoride and as an ingredient for condi-

tioning the fabric as to "hand" or "feel." Similarly, the selected moth-repelling ingredient is chosen for its additional mordanting or precipitating action, and to cooperate with and supplement the similar function of the aluminum sulphate. As to this latter, I have found that tartar emetic is very serviceable for this special combined purpose. This double salt of antimony has been found to possess inherent larvae-repelling properties, in addition to its mordant action. 10

It is a useful purpose of the present invention to utilize these materials, in appropriately combined form, not only for their own inherent qualities but also on account of their complementary mordanting functions. 15

As the requirement for variations in the desired "finish" of a given fabric necessitates modification of the relative quantities of the aluminum sulphate, a corresponding adjustment of the moth-repellent must be made to compensate for the loss of mordanting action by an increase in the quantity thereof within limits as will be readily appreciated as the general purposes of this invention are understood, and from a study of the specific exemplifications of the process as described herein.

The combination of the co-acting ingredients specified, namely, the highly water-soluble silico-fluoride, tartar emetic, and aluminum sulphate as exemplified in a preferred adaptation of the invention has been found to produce superior results both in effectiveness of mothproofing, respectively, moth-repelling action, and in rendering the treated fabrics suitable for market purposes.

In the practical application of the composition, it has also been found desirable to add an appropriately adapted quantity of dispersing agent such as a sulphonated higher aliphatic alcohol of the type of cetyl or lauryl alcohol, for example.

Having thus described my invention, I will now furnish specific exemplifications thereof. These examples are given in varied form for the purpose of illustrating the adaptation of the composition, having regard to the general requirements of the trade with respect to the quality, appearance and "hand" of particular materials treated.

## EXAMPLES

I. Fabrics, yarns, raw stock, etc., consisting entirely of animal fibres:

## 1. Fabrics

(a) About 100 lbs. of dyed fabric are circulated for about 20 minutes in a rinse bath (temperature 110° F.) to which has been added about 3 lbs. of a compound having the following composition: 54% silicofluoride, 28% tartar emetic, 60

17% aluminum sulphate, and 1% sulphonated higher alcohol.

(b) About 100 lbs. of dyed material are immersed for about two minutes in a standing bath to which has been added a solution of about 3 lbs. of a compound having the following composition: 54% silicofluoride, 28% tartar emetic, 17% aluminum sulphate, and 1% sulphonated higher alcohol in about 300 lbs. of cold water.

10 (c) About 100 lbs. of dyed fabric are "padded" for about 4 minutes in a jig bath to which has been added a solution of 2 to 4 lbs. of a compound having the following composition: 54% silicofluoride, 28% tartar emetic, 17% aluminum sulphate, and 1% sulphonated higher alcohol in about 400 lbs. of cold or tepid water.

## 2. Yarns or raw stock, etc.

(a) About 100 lbs. of yarn or raw stock are treated at 120° F. in the last bowl of the scouring bath previous to dyeing, or in the dyeing kettle after dyeing, by the addition of a solution containing about 400 lbs. of water and from 4 to 8 lbs. of a compound having the following composition: 54% silicofluoride, 28% tartar emetic, 17% aluminum sulphate, and 1% sulphonated higher alcohol.

II. Fabrics, yarns, or raw stock, etc., containing less than 25% of animal fibres and more than 75% of vegetable fibres:

### 1. Fabrics

(a) About 100 lbs. of dyed fabric are circulated for about 20 minutes in a rinse bath (temperature 110° F.) to which has been added about 4 lbs. of a compound having the following composition: 54% silicofluoride, 28% tartar emetic, 17% aluminum sulphate, and 1% sulphonated higher alcohol.

40 (b) About 100 lbs. of dyed material is immersed for about 2 minutes in a standing bath to which has been added about 4 lbs. of a compound having the following composition: 54% silicofluoride, 28% tartar emetic, 17% aluminum sulphate, and 1% sulphonated higher alcohol dissolved in about 400 lbs. of cold water.

45 (c) About 100 lbs. of dyed material is "padded" for about 4 minutes in a jig bath to which has been added about 1.5 to 3 lbs. of a compound having the following composition: 54% silicofluoride, 28% tartar emetic, 17% aluminum sulphate, and 1% sulphonated higher alcohol dissolved in about 300 lbs. of cold or tepid water.

## 2. Yarns or raw stock, etc.

(a) About 100 lbs. of yarn or raw stock are treated at 120° F. in the scouring bath previous to dyeing, or in the dyeing kettle after dyeing, by the addition of a solution consisting of about 300 lbs. of water and from 3 to 6 lbs. of a compound having the following composition: 54% silicofluoride, 28% tartar emetic, 17% aluminum sulphate, and 1% sulphonated higher alcohol.

55 III. Fabrics, yarns, or raw stock, etc., consisting wholly of animal fibres and intended for manufacture of finished goods requiring special "hand" or "feel."

### 1. Fabrics

(a) About 100 lbs. of dyed fabric are circulated for about 20 minutes in a rinse bath (temperature 110° F.) to which has been added about 3 lbs. of a compound having the following composition: 54% silicofluoride, 30% tartar emetic, 10% aluminum sulphate and 6% sulphonated higher alcohol.

5 (b) About 100 lbs. of dyed material are immersed for about 2 minutes in a standing bath to which has been added a solution of about 3 lbs. of a compound having the following composition: 54% silicofluoride, 30% tartar emetic, 10% aluminum sulphate and 6% sulphonated higher alcohol in about 300 lbs. of cold water.

(c) About 100 lbs. of dyed fabric are "padded" for about 4 minutes in a jig bath to which has been added a solution of 2 to 4 lbs. of a compound having the following composition: 54% silicofluoride, 30% tartar emetic, 10% aluminum sulphate and 6% sulphonated higher alcohol in about 400 lbs. of cold or tepid water.

## 2. Yarns or raw stock

(a) About 100 lbs. of yarn or raw stock are treated at 120° F. in a scouring bath previous to dyeing, or in the dyeing kettle after dyeing, by the addition of a solution consisting of about 400 lbs. of water and from 4 to 8 lbs. of a compound having the following composition: 54% silicofluoride, 30% tartar emetic, 10% aluminum sulphate, and 6% sulphonated higher alcohol.

From all of the foregoing examples, and the indications as to the manner of practicing desirable variations for specific purposes, those skilled in the art will be in a position to adapt the solutions to any desired requirement for particular purposes and fabrics. Thus, from the examples given for materials containing mixtures of animal and vegetable fibres, appropriate adaptations may be made for other mixtures of varying amounts of animal and vegetable fibres.

I claim:

1. A mothproofing composition which comprises essentially a member of the group consisting of magnesium silicofluoride and ammonium silicofluoride, and a comparatively small amount of tartar emetic.

40 2. A mothproofing composition which is composed essentially of about 50 per cent. of a member of the group consisting of magnesium silicofluoride and ammonium silicofluoride, about 30 per cent. of tartar emetic, an additional mordant, and a sulphonated higher alcohol.

3. A mothproofing composition composed essentially of about 50 per cent. of a member of the group consisting of magnesium silicofluoride and ammonium silicofluoride, about 30 per cent. of tartar emetic, about 10 to 17 per cent. of aluminum sulphate, and about 1 to 6 per cent. of a sulphonated higher alcohol.

4. The method of mothproofing a dyed textile fabric composed in substantial part of animal fibres, which comprises immersing the fabric in a dilute aqueous bath containing one of the group consisting of magnesium and ammonium silicofluorides, a lesser amount of tartar emetic, aluminum sulphate, and a wetting agent.

5. The method of mothproofing a textile fabric composed of animal or vegetable fibres which comprises immersing the fabric in a water bath containing in solution therein about 1 to 2 per cent. of a composition composed essentially of about 50 per cent. of a member of the group consisting of magnesium silicofluoride and ammonium silicofluoride, about 30 per cent. of tartar emetic, an additional mordant, and a wetting agent.

6. A mothproofing composition which comprises essentially a water-soluble silicofluoride and a less amount of tartar emetic.

15

35

40

60

70